

R. BURGER.  
MAKING DOUBLE WALLED VACUUM VESSELS.  
APPLICATION FILED JAN. 5, 1909.

918,503.

Patented Apr. 20, 1909.



Witnesses:  
May J. Mc Garry.  
Gwendolyn T. Porter.

Inventor  
Reinhard Burger  
By his Attorney Paul Benjamin

# UNITED STATES PATENT OFFICE.

REINHOLD BURGER, OF BERLIN, GERMANY.

## MAKING DOUBLE-WALLED VACUUM VESSELS.

No. 918,503.

Specification of Letters Patent.

Patented April 20, 1909.

Application filed January 5, 1909. Serial No. 470,864.

*To all whom it may concern:*

Be it known that I, REINHOLD BURGER, a subject of the German Emperor, residing at Berlin, Germany, have invented a certain 5 new and useful Improvement in Making Double-Walled Vacuum Vessels, of which the following is a specification.

The invention relates to the manufacture of double walled glass vacuum vessels, such 10 as bottles, and consists broadly in the process hereinafter described and comprising the steps more particularly pointed out in the claims.

In the accompanying drawings which are 15 all longitudinal sectional views—Figure 1 shows separately the glass cylinder which ultimately forms the outer wall of the bottle. Fig. 2 shows separately the glass cylinder which ultimately forms the inner wall of the 20 bottle. Fig. 3 shows the cylinder of Fig. 2 placed within the cylinder of Fig. 1, and the supporting plugs in place between the walls. Fig. 4 shows the two cylinders connected only at the end of the neck or mouth of the 25 now double walled vessel. Fig. 5 shows the same with one of the tubular projections closed. Fig. 6 shows the completed vessel with both tubular projections closed after exhaustion of the space between the double 30 walls.

Similar letters of reference indicate like parts.

I carry my process into effect in the following manner: The glass cylinder A, which 35 is to form the outer wall of the vacuum vessel, is usually received from the glass blowers in the shape illustrated in Fig. 1, in which case, the upper portion B is cut off on the line a, a, in order to produce a cylinder of the desired 40 shape having an open end at C and a rounded bottom end at D. The glass cylinder E, which is of less diameter than cylinder A and is to form the inner wall of the vacuum vessel, is usually received from the glass blowers 45 in the shape illustrated in Fig. 2, that is, with a long body portion F and an open neck G. Upon the rounded bottom C of the outer cylinder A, I form two small projecting tubes H, I. I then place the cylinder E within the 50 cylinder A, as shown in Fig. 3, and in any suitable way introduce into the space between said cylinders, bodies or plugs J, preferably made of asbestos paper or other yielding heat insulating material. Said plugs 55 may be attached to the surface of the inner cylinder E in any suitable manner, such for

instance, in the way set forth in U. S. Letters Patent No. 888,783, granted to me May 26, 1908, before the said cylinder E is inserted into the cylinder A, or by adhesion; or they 60 may be inserted into the space between the cylinders after said cylinders are put together and then retained in place by engagement with the walls. For convenience in handling and spacing, they may be connected 65 by a ring K of wire or cord. A lip L may also be formed at the open end of the neck of cylinder E, if desired. The two cylinders are next fused together at their mouths, as shown in Fig. 4, and suitably molded to 70 shape, thus producing a double walled vessel. In order to fill the pores of the glass, a silvering solution or other suitable coating may be introduced through one of said projections into the space between the walls, and a coating 75 of silver or other material thus applied. One of the projections, as I, is then sealed, Fig. 5, and substantially a vacuum is produced in the said space by any suitable device applied to the remaining projection H. The 80 last named projection is then sealed, thus completing the vessel, as shown in Fig. 6.

I claim:

1. The process of making glass vacuum vessels which consists in, first, placing within 85 a glass cylinder closed at one end and open at the opposite end, a second cylinder of less diameter open at one end and closed at the other end, so that a space will be formed between said cylinders and introducing supporting bodies into said space: second, fusing said cylinders together at their open ends: third, producing substantially a vacuum in 90 said intermediate space, and fourth, sealing 95 the opening in said outer cylinder.

2. The process of making glass vacuum vessels which consists in, first, forming on the closed end of a glass cylinder, open at the opposite end, a tubular projection: second, inserting in said cylinder a second cylinder of less diameter open at one end and closed at the other end, so that a space will be formed between said cylinders: third, inserting supporting bodies in said space: fourth, fusing 100 said cylinders together at their open ends: fifth, producing substantially a vacuum in 105 said intermediate space, and sixth, sealing said tubular projection.

3. The process of making glass vacuum 110 vessels which consists in, first, forming on the closed end of a glass cylinder, open at the op-

posite end, two tubular projections: second, inserting in said cylinder a second cylinder of less diameter open at one end and closed at the other, so that a space will be formed between said cylinders: third, inserting supporting bodies in said space: fourth, fusing said cylinders together at their open ends: fifth, introducing a coating solution into said space: sixth, closing one of said tubular pro-

jections: seventh, producing substantially a <sup>10</sup> vacuum in said space, and eighth, closing said remaining tubular projection.

In testimony whereof I have affixed my signature in presence of two witnesses.

REINHOLD BURGER.

Witnesses:

WOLDEMAR HAUPT,  
HENRY HASPER.